

# United States Patent Office

3.595.662

Patented July 27, 1971

1

3.595.662

**3,393,002**  
**LIGHT-SENSITIVE MATERIAL**

**LIGHT-SENSITIVE MATERIAL**  
Jozef Frans Willems, Wilrijk, and Robrecht Julius Thiers,  
Brasschaat, Belgium, assignors to Gevaert-Agfa N.V.,  
Mortsel, Belgium

Morsel, Belgium  
No Drawing. Filed Dec. 7, 1967. Ser. No. 688,670

NO Drawing. Filed Dec. 7, 1967, Ser. No. 668,670  
Claims priority, application Great Britain, Mar. 6, 1967.

10,372/67  
Int. Cl. G03c 1/34

## 12 Claims

## ABSTRACT OF THE DISCLOSURE

A light-sensitive material comprising a silver halide emulsion layer and containing a mercury(II) chelate of a (poly)amino-(poly)carboxylic acid in the form of the acid or a water-soluble salt is described. The chelate exerts a stabilizing and fog-inhibiting action upon the light-sensitive material without causing appreciable desensitization.

This invention relates to improved light-sensitive silver halide emulsions.

Light-sensitive silver halide emulsions are in general characterised by their sensitivity, gradation and fog.

As is well-known, sensitivity, gradation and fog are determined by the way in which the silver halide emulsion is prepared and by the use of special chemical ingredients effecting a desired improvement or result. Addenda to the emulsion, which are of particular importance for the stability of the light-sensitive characteristics of a silver halide emulsion are the so-called "stabilizers."

Stabilizers or antifoggants protect the light-sensitive silver halide emulsions against spontaneous formation and growth of fog known as chemical fog during prolonged storage or storage at high temperatures and humidities or during development to maximum contrast and speed. Indeed, the fog increases with the degree and temperature of development, and, in constant development circumstances, with the time the light-sensitive emulsion is stored and with the temperature and the relative humidity of the atmosphere wherein the emulsion is stored. It is evident that a light-sensitive emulsion should be obtained which is as stable as possible at high temperature and high relative humidity for instance in view of its use in tropical countries.

It is known to protect light-sensitive silver halide emulsions against the growth of chemical fog during storage by addition of stabilizers of the triazolopyrimidine type (azaindolizines). Heterocyclic thioxo and mercapto compounds too have been proposed for this purpose but show the disadvantage of impairing the sensitivity and gradation. The same disadvantageous influence on the sensitivity occurs with the known mercury salts, addition complexes of mercury salts with amines, organic mercury salts and heterocyclic mercury compounds. Indeed, these compounds, when used in the concentration necessary for obtaining a sufficient antifogging action, have a considerable desensitizing effect.

It is also known that emulsions stabilised with compounds of the triazolopyrimidine type still show a tendency to fog formation in extreme storage circumstances i.e. at very high temperatures and humidities and in extreme development circumstances e.g. rapid processing at elevated temperatures. The addition to these emulsions of the above known mercury compounds reduces the fogging tendency but, as mentioned above, at the cost of a reduction of the sensitivity.

It has now been found that when incorporating in a light-sensitive material comprising a silver halide emul-

2

sion layer mercury(II) chelates of (poly)amino-(poly) carboxylic acids, in acid form or in the form of a water-soluble salt, these compounds exert a stabilizing and fog-inhibiting action upon said photographic light-sensitive material without causing an appreciable desensitization thereof.

Moreover, it has been found that these mercury(II) chelates are very suitable for use in combination with stabilizers of the triazolopyrimidine type, particularly in extreme storage and development circumstances in order to reduce the fogging tendency of the light-sensitive emulsion without giving rise to an appreciable desensitization thereof.

As will be illustrated further on, the mercury(II) chelates of (poly)amino(poly)carboxylic acids can be prepared by allowing to react a water-soluble mercury (II) salt (chloride, cyanide, acetate, etc.) with a (poly)amino(poly)carboxylic acid or water-soluble salt thereof or by treating the sequestering compound, in acid form or 20 in the form of a water-soluble salt, with mercury(II) oxide until the mercury oxide has dissolved completely (cf. H. Möhrle, Archiv der Pharmazie 299 (1966) 529).

Examples of suitable (poly)amino(poly)carboxylic acid sequestering compounds for reaction with a mercury (II) salt or mercury(II) oxide to form the corresponding mercury(II) chelates as well as details about the preparation of said sequestering compounds can be found in *Ind. Chim. Belg.*, T XXI (1956), pp. 338-346 and in *Ind. Chim. Belg.*, T XXIII (1958), pp. 1105-1115.

Particularly suitable (poly)amino (poly)carboxylic acids for forming in acid or salt form with a mercury(II) salt or mercury(II) oxide the corresponding mercury(III) chelates can be represented by the following non-limitative general formula:



wherein:

L stands for alkylene including substituted alkylene e.g. hydroxyalkylene, cycloalkylene including substituted cycloalkylene or alkylene interrupted by one or more hetero atoms, such as an oxygen atom.

45  $x$  represents 0, 1 or 2.

R stands for lower alkylene e.g. methylene and ethylene including substituted lower alkylene, e.g. alkylene substituted by alkyl, aryl, aralkyl, including substituted alkyl, aryl and aralkyl, and

50 each of  $R_1$  and  $R_2$  (the same or different) stands for hydrogen, lower alkyl including substituted lower alkyl, aralkyl including substituted aralkyl or aryl including substituted aryl; examples of substituted alkyl groups for  $R_1$  and for  $R_2$  are alkyl substituted with hydroxyl, 55 halogen, alkoxy, carbamoyl, amino, substituted amino e.g. dihydroxyalkylamino, epoxy, carboxyl, sulpho, phosphono, mercapto, alkylmercapto, alkoxycarbonyl, a nitrogen-containing heterocyclic ring e.g. pyridyl and examples of substituted aryl groups and aralkyl groups 60 for  $R_1$  and/or  $R_2$  are: aryl and aralkyl substituted by hydroxyl, halogen, alkyl, alkoxy, nitro, carboxyl and sulpho.

65 The following is a non-limitative list of examples of (poly)amino(poly)carboxylic acids corresponding to the above general formula:





The following preparations illustrate more particularly how the mercury(II) chelates of the (poly)amino-(poly)carboxylic acids can be prepared.

**5**  
**PREPARATION 1**

**Mercury(II) chelate of compound 1**

To a solution of 38 g. (0.1 mole) of ethylenediamine N,N,N',N'-tetraacetic acid disodium salt dihydrate in 200 ml. of water 21.5 g. (0.1 mole) of mercury(II) oxide are added portionwise at room temperature with stirring. The mercury(II) oxide dissolves gradually. After 3 hours the aqueous solution obtained is filtered, evaporated under reduced pressure at 50° C. and the solid product formed is dried under reduced pressure at 50° C. in a drying oven. The product obtained is a white amorphous powder which is soluble in water. Yield: 50 g.

**PREPARATION 2**

**Mercury(II) chelate of compound 15**

To a solution of 20.9 g. (0.055 mole) of ethyleneglycol bis(2-aminoethyl), N,N,N',N'-tetraacetic acid in 400 ml. of water is added at room temperature a solution of 4.4 g. (0.11 mole) of sodium hydroxide in 50 ml. of water. At the same temperature, 10.8 g. (0.05 mole) of mercury(II) oxide are then added portionwise with stirring. The mercury(II) oxide dissolves gradually. After 3 hours the aqueous solution obtained is filtered, evaporated under reduced pressure at 50° C. and the solid product formed is dried under reduced pressure at 50° C. in a drying oven. The product obtained is an amorphous powder which is soluble in water. Yield: 31 g.

**PREPARATION 3**

**Mercury(II) chelate of compound 8**

To a solution of 43.2 g. (0.11 mole) of diethylenetri-amine-N,N,N',N',N"-pentaacetic acid in 400 ml. of water is added at room temperature a solution of 13.2 g. (0.33 mole) of sodium hydroxide in 50 ml. of water. At the same temperature, 21.6 g. (0.1 mole) of mercury(II) oxide are then added portionwise with stirring.

The mercury(II) oxide dissolves gradually. After 3 hours the aqueous solution formed is filtered, evaporated under reduced pressure at 50° C. and the solid product formed is dried under reduced pressure at 50° C. in a drying oven. The product obtained is a white amorphous powder which is soluble in water. Yield: 75 g.

**PREPARATION 4**

**Mercury(II) chelate of compound 4**

To a solution of 30.5 g. (0.11 mole) of N-(2-hydroxyethyl)-ethylenediamine-N,N',N'-triacetic acid in 400 ml. of water is added at room temperature a solution of 4.4 g. (0.11 mole) of sodium hydroxide in 50 ml. of water. At the same temperature, 21.6 g. (0.1 mole) of mercury(II) oxide are then added portionwise with stirring. The mercury(II) oxide dissolves gradually. After 3 hours the aqueous solution obtained is filtered, evaporated under reduced pressure at 50° C. and the solid product formed is dried under reduced pressure at 50° C. in a drying oven. The product obtained is a white amorphous powder which is soluble in water. Yield: 55 g.

**PREPARATION 5**

**Mercury(II) chelate of compound 10**

To a solution of 19.8 g. (0.055 mole) of ethylenediamine,N,N'-di(o-hydroxyphenyl-acetic acid) in 400 ml. of water is added at room temperature a solution of 4.4 g. (0.11 mole) of sodium hydroxide in 50 ml. of water. At the same temperature, 10.8 g. (0.05 mole) of mercury(II) oxide are added portionwise with stirring to the brown solution. The mercury(II) oxide dissolves gradually. After 3 hours the aqueous solution obtained is filtered, evaporated under reduced pressure at 50° C. and the solid product formed is dried under reduced pressure at 50° C. in a drying oven. The product obtained is a brown amorphous powder which is soluble in water. Yield: 33 g.

**6**

As compared with the known mercury compounds used as stabilizers the mercury(II) chelates according to the present invention when used in the appropriate concentration do not cause or only to a slight extent a decrease in sensitivity.

5 The antifoggants according to the present invention are particularly suitable for use in combination with compounds which sensitize the emulsion by development acceleration for example compounds of the polyoxyalkylene 10 type such as alkylene oxide condensation products as described among others in U.S. Pats. 2,531,832 and 2,533,990, in U.K. Pats. 920,637, 940,051, 945,340 and 991,608 and in Belgian Pat. 648,710 and onium derivatives of amino-N-oxides as described in U.K. patent application 42,592/65.

15 The stabilizers according to the invention can also be used in combination with other known stabilizers for instance with heterocyclic nitrogen containing thioxo compounds such as benzothiazoline-2-thione and 1-phenyl-2-tetrazoline-5-thione, with other mercury compounds and, as said above, preferably with compounds of the hydroxytriazolopyrimidine type (azaindolizines).

20 The stabilizers according to the present invention may be incorporated into any type of light-sensitive material comprising a silver halide emulsion layer e.g. a spectrally sensitized or non-sensitized emulsion layer, an X-ray emulsion layer, and an emulsion layer sensitive to infrared radiation. They may be incorporated into high-speed negative materials as well as into rather low speed positive 25 materials. Various silver salts may be used as light-sensitive salt e.g. silver bromide, silver iodide, silver chloride, or mixed silver halides e.g. silver chloro-bromide or silver bromo-iodide.

30 The silver halides are dispersed in the common hydrophilic colloids such as gelatin, casein, zein, polyvinyl alcohol, carboxymethylcellulose, alginic acid, etc., a gelatin being however favoured.

35 The stabilizing agents are generally incorporated into the silver halide emulsion layer of the light-sensitive material; they may be added to the emulsion during no matter what step of emulsion preparation; however, they are preferably added to the photographic emulsion after chemical ripening and just before coating of the emulsion. The addenda according to the present invention are incorporated into the photographic emulsions according to 40 the methods well known in emulsion preparation, e.g. in the form of a solution in water.

45 Instead of incorporating the compounds of the invention into the emulsion layer they can also be incorporated 50 into a water-permeable layer e.g. a gelatin covering layer or intermediate layer.

The amount of mercury(II) chelate employed in the 55 light-sensitive silver halide material depends on the particular type of emulsion and the desired effect and can vary within very wide limits. The optimum amount of mercury(II) chelate to be added can be determined for each particular type of emulsion in a very simple way by application of the usual tests. Usually said compounds are employed in a ratio of about 0.1 mg. to about 30 mg. per 60 mole of silver halide, preferably from 0.5 to 10 mg. per mole of silver halide.

65 The light-sensitive emulsions may be chemically as well as optically sensitized. They may be chemically sensitized by effecting the ripening in the presence of small amounts of sulphur containing compounds such as allyl-thiocyanate, allyl thiourea, sodium thiosulphate, etc. The emulsions may also be sensitized by means of reductors for instance tin compounds as described in our French 70 patent specification 1,146,955 and in our Belgian patent specification 568,687, imino-amino methane sulphonic acid compounds as described in our British patent specification 789,823 and small amounts of noble metal compounds such as of gold, platinum, palladium, iridium, 75 ruthenium and rhodium.

Other addenda such as hardening agents, wetting agents, plasticizers, colour couplers, developing agents and optical sensitizers can be incorporated into the emulsion in the usual way.

The following examples illustrate the present invention.

#### EXAMPLE 1

A high sensitive gelatino silver bromoiodide emulsion ( $\pm 4.5$  moles percent of iodide) is divided into nine aliquot portions A, B, C, D, E, F, G, H and I.

To each of these emulsion portions, except for one (emulsion A) is added per mole of silver halide one of the following mercury (II) compounds in the amount indicated:

emulsion B:  $0.6 \times 10^{-2}$  millimole (1.5 mg.) of mercury (II) cyanide

emulsion C:  $1.2 \times 10^{-2}$  millimole (3 mg.) of mercury (II) cyanide

emulsion D:  $0.6 \times 10^{-2}$  millimole (4 mg.) of the mercury (II) chelate of compound 8 trisodium salt

emulsion E:  $0.6 \times 10^{-2}$  millimole (3 mg.) of the mercury (II) chelate of compound 4 sodium salt

emulsion F:  $0.6 \times 10^{-2}$  millimole (3.7 mg.) of the mercury (II) chelate of compound 15 disodium salt

emulsion G:  $1.2 \times 10^{-2}$  millimole (7.5 mg.) of the mercury (II) chelate of compound 15 disodium salt

emulsion H:  $0.6 \times 10^{-2}$  millimole (3.1 mg.) of the mercury (II) chelate of compound 1 disodium salt

emulsion I:  $1.2 \times 10^{-2}$  millimole (6.2 mg.) of the mercury (II) chelate of compound 1 disodium salt.

The nine emulsions are then coated on a subbed cellulose triacetate support and dried whereupon the nine materials thus obtained are stored for 5 days in an atmosphere of 57°C. and 34% of relative humidity.

The stored materials as well as nine identical freshly prepared materials are exposed and developed for 5 minutes at 20°C. in a developing bath with the following composition:

Water—800 ccs.

p-Monomethylaminophenol sulphate—1.5 g.

Sodium sulphite (anhydrous)—50 g.

Hydroquinone—6 g.

Sodium carbonate (anhydrous)—32 g.

Potassium bromide—2 g.

Water up to 1000 ccs.

After the treatment in a stop bath, rinsing and fixing of the materials the following sensitometric results are obtained.

| Material | Freshly prepared materials |           |                         | Stored materials |           |                         |
|----------|----------------------------|-----------|-------------------------|------------------|-----------|-------------------------|
|          | Fog                        | Gradation | Relative speed, percent | Fog              | Gradation | Relative speed, percent |
| A-----   | 0.11                       | 1.62      | 100                     | 0.46             | 1.38      | 118                     |
| B-----   | 0.09                       | 1.67      | 71                      | 0.11             | 1.51      | 87                      |
| C-----   | 0.09                       | 1.61      | 33                      | 0.09             | 1.61      | 37                      |
| D-----   | 0.10                       | 1.64      | 89                      | 0.10             | 1.61      | 142                     |
| E-----   | 0.08                       | 1.75      | 89                      | 0.09             | 1.71      | 96                      |
| F-----   | 0.09                       | 1.74      | 94                      | 0.13             | 1.56      | 145                     |
| G-----   | 0.08                       | 1.70      | 68                      | 0.09             | 1.67      | 76                      |
| H-----   | 0.09                       | 1.48      | 96                      | 0.20             | 1.54      | 136                     |
| I-----   | 0.05                       | 1.61      | 61                      | 0.04             | 1.60      | 74                      |

The speed is given in relative values (i.e. in percent) in respect of the absolute speed of an emulsion to which no mercury (II) compound was added. From this example it clearly appears that for the same fog-level the mercury (II) chelates according to the invention have a markedly less desensitizing effect than the common organic mercury salts.

#### EXAMPLE 2

A gelatino silver bromoiodide emulsion (0.20 mole percent of iodide) comprising per mole of silver halide 400 mg. of 5-methyl-7-hydroxy-s-triazolo-[1,5-a]-pyrimidine as stabilizer and per litre of emulsion 1 g. of saponin as coating aid, is divided into 3 aliquot portions.

To emulsion portion B is added 1 mg. of mercury (II) cyanide per mole of silver halide whereas to emulsion portion C 1.5 mg. of the mercury (II) chelate of compound 1 disodium salt is added per mole of silver halide. To emulsion portion A no mercury (II) compound is added.

The three emulsions are coated on a subbed cellulose triacetate support and the emulsion layers are then overcoated with a gelatin antistress layer.

Thereupon the said three materials are developed at 20°C. in a common X-ray developer having the following composition:

Water—800 ccs.

p-Monomethylaminophenol hemisulphate—4 g.

Hydroquinone—10 g.

Anhydrous sodium sulphite—65 g.

Anhydrous sodium carbonate—45 g.

Potassium bromide—5 g.

Water up to 1000 ccs.

The fog produced in the respective materials after a development time of 4 and 8 min. is listed in the following Table 1.

TABLE 1

| Material | Fog produced after a development time of— |        |
|----------|-------------------------------------------|--------|
|          | 4 min.                                    | 8 min. |
| A-----   | 0.17                                      | 0.27   |
| B-----   | 0.16                                      | 0.19   |
| C-----   | 0.13                                      | 0.13   |

Three identical materials A, B and C are kept for 36 hours in an atmosphere of 57°C. and 34% of relative humidity and then developed for 4 min. at 20°C. in the same developer. The fog produced in the respective materials is listed in Table 2.

TABLE 2

| Material: | Fog produced |      |
|-----------|--------------|------|
|           | A            | B    |
| A-----    | 0.39         |      |
| B-----    |              | 0.20 |
| C-----    |              | 0.13 |

We claim:

1. Photographic material comprising a support and at least one light-sensitive silver halide emulsion layer comprising in said emulsion layer at least one mercury (II) chelate of a (poly)amino(poly)carboxylic acid in acid form or in the form of a water-soluble salt, said chelate being present in an amount sufficient to stabilize said material with regard to fogging.

2. Photographic light-sensitive silver halide material according to claim 1, wherein said (poly)amino(poly)carboxylic acid corresponds to the following general formula:



wherein:

L stands for alkylene including substituted alkylene and alkylene interrupted by one or more hetero atoms or cycloalkylene including substituted cycloalkylene,

x represents 0, 1 or 2,

R stands for lower alkylene including substituted lower alkylene, and

each of  $R_1$  and  $R_2$  (the same or different) stands for hydrogen, lower alkyl including substituted lower alkyl, aralkyl including substituted aralkyl or aryl including substituted aryl.

3. Photographic light-sensitive silver halide material according to claim 1, wherein said mercury(II) chelate is present in an amount of from 0.1 mg. to 30 mg. per mole of silver halide.

4. Photographic light-sensitive silver halide material according to claim 1, wherein said material also comprises a hydroxytriazolopyrimidine stabilizer.

5. Photographic light-sensitive silver halide material according to claim 1, wherein said material also comprises a polyoxyalkylene development accelerator.

- 6.** Photographic light-sensitive silver halide material according to claim 1, wherein said emulsion layer is a gelatino silver halide emulsion layer.

7. Photographic material comprising a support and at least one light-sensitive silver halide emulsion layer comprising in a water permeable layer coated at the same side of the support as the emulsion layer at least one mercury (II) chelate of a (poly)amino(poly)carboxylic acid in acid form or in the form of a water-soluble salt, said chelate being present in an amount sufficient to stabilize said material with regard to fogging.

8. Photographic light-sensitive silver halide material according to claim 7, wherein said (poly)amino(poly)-carboxylic acid corresponds to the following general formula:



wherein:

L stands for alkylene including substituted alkylene and alkylene interrupted by one or more hetero atoms or cycloalkylene including substituted cycloalkylene,

$x$  represents 0, 1 or 2,

R stands for lower alkylene including substituted lower alkylene, and each of  $R_1$  and  $R_2$  (the same or different) stands for hydrogen, lower alkyl including substituted

lower alkyl, aralkyl including substituted aralkyl or aryl including substituted aryl.

9. Photographic light-sensitive silver halide material according to claim 7, wherein said mercury(II) chelate is present in an amount of from 0.1 mg. to 30 mg. per mole of silver halide.

10. Photographic light-sensitive silver halide material according to claim 7, wherein said material also comprises a hydroxytriazolopyrimidine stabilizer.

- a hydroxylazolopyrimidine stabilizer.

11. Photographic light-sensitive silver halide material according to claim 7, wherein said material also comprises a polyoxyalkylene development accelerator.

- ## 12. Photographic light-sensitive silver halide material

### References Cited

UNITED STATES PATENTS

|           |         |                    |         |
|-----------|---------|--------------------|---------|
| 2,273,562 | 2/1942  | Davey et al. ----- | 96-109  |
| 2,531,832 | 11/1950 | Stanton -----      | 96-66   |
| 2,533,990 | 12/1950 | Blake -----        | 96-66.3 |
| 2,666,700 | 1/1954  | Baldsiefen -----   | 96-107  |
| 2,751,299 | 6/1956  | Carroll -----      | 96-107  |
| 3,161,515 | 12/1964 | Welsh -----        | 96-109  |

## FOREIGN PATENTS

574.802 4/1959 Canada 96-107

20 WILLIAM D. MARTIN, Primary Examiner

T. G. DAVIS, Assistant Examiner

U.S. CL X R

96—88, 107